

F. MÂNGE & M. J. T. BALS.  
MANUFACTURE OF MATCHES.  
APPLICATION FILED SEPT. 4, 1913.

1,102,158.

Patented June 30, 1914.

*Fig. 1.*



*Fig. 2.*



Witnesses  
A. F. Schilling  
J. M. Kenoch

Inventors  
Frédéric Mângé &  
Maximilian Joseph  
Theodor Bals  
by Paul Schilling

Attorney.

# UNITED STATES PATENT OFFICE.

FRÉDÉRIC MANGE AND MAXIMILIAN JOSEPH THEODOR BALS, OF PARIS, FRANCE.

## MANUFACTURE OF MATCHES.

1,102,158.

Specification of Letters Patent. Patented June 30, 1914.

Application filed September 4, 1913. Serial No. 788,134.

To all whom it may concern:

Be it known that we, FRÉDÉRIC MANGE, a citizen of the Swiss Republic, and MAXIMILIAN JOSEPH THEODOR BALS, a subject of the German Emperor, both residing at Paris, France, have invented certain new and useful Improvements in the Manufacture of Matches, of which the following is a specification.

10 The present invention has reference to improvements in the manufacture of matches, and it relates more particularly to a procedure according to which match-wood splints of a length of two or more matches 15 are suitably bundled-up and are then severed into bundles of single match length in such manner that the cut ends are roughened or frayed for the purpose of enabling them to more readily take up the impregnating and 20 tipping compositions. The bundles of single match length are then suitably impregnated and tipped, if desired at both ends, and are opened-up for boxing just prior to the ensuing drying process being completed. 25 The invention will now be described in detail, reference being had to the accompanying drawing, in which—

Figure 1 shows a side view of a device for clamping the match-wood splints during the 30 cutting operation; Fig. 2 shows a front view thereof.

According to our invention a plurality of splints of match-wood, each of a length of two or more matches of ordinary size, are 35 bundled-up in direct lateral contact with each other and held in this compacted state in any suitable manner, for instance by wire or other ligatures being placed around, or by being blocked within a clamping device, 40 such as shown, by way of example, in Figs. 1 and 2.

This device consists of a housing 1, into which are equidistantly fitted the frames 2, whose top members 3 are vertically adjustable thereon by means of the hinged lock-bolts 4. The bundle or block of matches 5 is placed in said frames which grip it at intervals of a match length apart and for as many match lengths as there are clamping 50 frames (nine in the drawing), and the splint strips are then severed into sections of match length by being cut or sawed, the knives or saw blades entering between each two frames 2, either successively or simultaneously. Or the splints are pressed into a suitable compacting device, and are then 55 successively presented thereby in sections of single match length; whereupon each such section is tied-up, wired or frame-clamped, and then severed from the main bundle. 60 During the cutting operation wood dust works into the interstices between the individual splints, which is a very valuable feature, inasmuch as now the impregnating and tipping ingredients cannot penetrate far 65 between the splints, which greatly reduces the amount of the compositions required for preparing a given number of matches compared to the old procedures. Furthermore the sawing operation tends to roughen or 70 fray the splint ends, which greatly enhances the capacity of the wood for absorbing the respective compositions, and for this purpose it has been found of advantage to use dulled cutting tools for severing the sections 75 from the main bundle. The thus severed small bundles, which are still held compacted by the wire hoops or the clamping frames, are now subjected to a temperature of about 120° for from 6-8 hours. They can then be 80 primed with a thin paste of flame transmitting medium, for instance powdered sulfur in gum tragacanth solution. When aspen or several other American woods are used, it suffices to saturate the roughened flame ends 85 of the splints with solutions of oxygen carriers, for instance chlorate of potash in gum tragacanth solution. Next, a suitable, thin but gluey igniting composition is applied in 90 well known manner. Comparatively little 90 of the composition will adhere to the frayed splint ends, owing to the latter being held close together and the sifted-in wood dust preventing the composition from "creeping" along the splints. The tipped bundles 95 are then dried in suitable manner. Just prior to completed drying the bundles are 100 opened-up by removal of the tying means, for separating the individual matches for further manipulations. The falling-apart of the bundle into single matches will readily take place owing to the ends of the splints swelling-up by the taken-up liquid, which in connection with the tying-up means causes strong tensions being set up in 105 the bundle. The loose matches are then left to complete their drying, without further heat having to be applied. The matches are now ready for boxing, an operation which 110 will proceed very quickly, owing to the fact that the matches will show no appreciable thickening or lengthening at the tipped ends,

and owing to this absence of enlarged heads or tips a considerably greater number of these matches can be packed into a given box than would be possible in the case of the old style matches with globularly extending tips.

What we claim is:—

1. That improvement in the art of match-making which comprises assembling long splints of match wood into direct lateral contact with each other to form a bundle, binding-up such bundle at match length intervals, severing the bundle into sections of a match length between such bindings, applying chemicals to the ends of the tightly bound together splints the application of the chemicals to individual splints being restricted to the end face of the splint by the proximity of the adjacent splints and unloosening the binding before the chemicals have completely dried or set.
2. That improvement in the art of match-

making which comprises assembling long splints of match-wood into direct lateral contact with each other to form a bundle, 25 binding-up such bundle at match length intervals, severing the bundle into sections of a match length between such bindings in such manner as to make rough or frayed the severed splint ends, applying chemicals 30 to the ends of the tightly bound together splints, the application of the chemicals to individual splints being restricted to the end face of the splint by the proximity of the adjacent splints and unloosening the binding 35 before the chemicals have completely dried and set.

In testimony whereof we affix our signatures in the presence of two witnesses.

FRÉDÉRIC MANGE.

MAXIMILIAN JOSEPH THEODOR BALS.

Witnesses:

HANSON C. COXE,

JOHN BAKER.

---

Copies of this patent may be obtained for five cents each, by addressing the "Commissioner of Patents, Washington, D. C."